

# UNITED STATES PATENT OFFICE.

ALFRED O. TATE, OF MONTREAL, QUEBEC, CANADA, ASSIGNOR TO TATE ELECTROLYTIC WATERPROOFING COMPANY, INCORPORATED, OF NEW YORK, N. Y., A CORPORATION OF NEW YORK.

## METHOD OF WATERPROOFING FIBROUS MATERIALS.

1,228,987.

Specification of Letters Patent.

Patented June 5, 1917.

No Drawing.

Application filed October 27, 1916. Serial No. 127,997.

*To all whom it may concern:*

Be it known that I, ALFRED O. TATE, a subject of the King of Great Britain, residing at Montreal, in the Province of Quebec, 5 Dominion of Canada, have invented certain new and useful Improvements in Methods of Waterproofing Fibrous Materials.

My invention relates to the art of waterproofing fibrous materials by the suspension or elimination of the capillary action of the fibers of a fabric, thus preventing the penetration or absorption of moisture, in the general manner described in my prior Patent, No. 933,861, issued to me September 15 14, 1909. This invention is an improvement upon the method of my prior patent and also upon the process described by me in my pending application Serial No. 879,872, filed December 31, 1914.

Some of the objects of my invention are to improve the process of my prior Patent No. 933,861; to effect a practically permanent suspension or elimination of capillary action in fibrous materials, thus effecting a substantial waterproofing of the fabric without at the same time appreciably decreasing its original porosity or ventilating qualities; to effect waterproofing of said materials without appreciably changing their 25 texture or color; to render materials so treated practically stainproof; to fix dies in fabrics treated with unfixed dies; and to obtain the foregoing objects by means of a process which is simple, economical and rapidly operated.

Generally speaking, my invention consists in the permeation or impregnation of the material to be treated which may be in the form of a fabric or thread, with a saponaceous substance, and the incorporation therein of a metallic acetate and a metallic hydroxid. I thus incorporate in the material treated a material which is water-repelling but soluble, and also two substances, 45 one at least of which is insoluble in water. These three substances combine to form an insoluble waterproof substance with which the fibers of the material are impregnated to the extent that capillary action is more or less entirely eliminated.

Materials treated according to my improved process are practically waterproof and remain so even after having been subjected to friction or wear, or boiling for pe-

riods long enough to indicate the practically permanent nature of their non-absorbent qualities. Boiling provides one of the severest tests for waterproofing, since the heat and molecular friction incident thereto produce effects on the material which can be realized in no other manner known to me.

I find that sodium palmitate, a constituent of white Castile soap, aluminum acetate and aluminum hydroxid are suitable substances for the practice of my invention. I find that sodium palmitate is desirable because of its chemical properties and because of its physical properties, in that it may be rendered sufficiently fluid to enter capillaries of any fiber with which I am familiar. 70 Aluminum acetate and aluminum hydroxid are preferably used because, when combined with the sodium palmitate, a practically colorless waterproof and non-absorbent substance is formed, thus preserving the original color of the material treated. These substances also have important physical and chemical properties, by reason of which they lend themselves to the practice of my process.

While I have stated these substances to be those which I at present prefer in the practice of my invention, it will be evident to those skilled in the art that other substances might be substituted for those named as, for instance, the acetates and hydroxids of other metals. It is also evident that saponaceous substances, other than palmitate of soda, may be found suitable to the practice of my invention, and I do not, therefore, desire to confine myself to the use of any of the three substances particularly described, but intend to cover in my claims all equivalent methods of practising my invention.

In practising my improved process, the material treated is first saturated with a solution of the saponaceous substance, preferably sodium palmitate, and then passed between two electrodes, which may be in the form of conducting rolls, although electrodes of any other suitable shape may be used. One electrode or roll represents the positive, and the other the negative, element of an electrolytic cell through which a current of electricity flows. The positive 105 electrode or roll should be of the metal, the hydroxid of which it is desired to incorporate. The negative roll or electrode may be

of any suitable material. When using aluminum acetate and aluminum hydroxid I usually make both rolls of the metal aluminum. While the material under treatment is passing between the electrodes, I apply a solution of the metallic acetate, such as aluminum acetate, in any suitable manner, as by spraying on the surface of the negative roll. At the same time, a nascent metallic hydroxid, as for instance, aluminum hydroxid, is introduced by electrolytic precipitation from the surface of the positive metallic roll. I find that the simultaneous application of the aluminum acetate and the electric current produces results which are far superior to the results obtained by any waterproofing process heretofore known to me. It will be understood that the number of pairs of electrodes or rolls may be increased as desired, for the purpose of augmenting the quantity of non-absorbent substance introduced into the fabric, in the same manner described above. After passing through the electrodes the material is washed and dried in any suitable manner.

It will be understood that the strength of the solutions, the time of treatment, and the value of the current may be varied, depending in great measure upon the nature, quality and thickness of the material to be treated. These values may best be determined by test. For the purpose of giving values which I have found operative, I will describe those I prefer to use in the case of woolens, such as ordinarily used for clothing, although these values may vary from those stated. In the case of woolens of this type, I find that a satisfactory degree of waterproofing is obtained by using a solution of sodium palmitate in the proportions of one-half ounce of white Castile soap containing sodium palmitate to one gallon of water, a solution of aluminum acetate of 13 degrees T. W., and current density of about five amperes per linear foot of cylindrical electrode surface. In this case the goods are passed between the electrodes at the rate of about three feet per minute, the rolls used being seven inches in diameter, the positive roll being aluminum and the negative roll being graphite.

The action of the current in the above described process is important in producing a superior product, for in addition to any aluminum hydrate, and aluminum palmitate that may be ordinarily precipitated by the chemical action of the aluminum acetate on the sodium palmitate present in the cloth, the said current acts in passing between the aluminum electrodes to not only hasten this true chemical precipitation, but also to electrolytically precipitate on the fibers of the cloth what I call a chemical excess of aluminum hydrate, which is independent of any chemical proportions of sodium palmitate and aluminum acetate present; as this said chemical excess of aluminum hydrate is water repellent it serves to produce waterproofing qualities in the fabric being treated of a very high order.

Not only does the simultaneous application of the electric current thus provide a quicker chemical precipitation of aluminum palmitate and aluminum hydrate, and a chemical excess of a valuable water repelling material on the individual fibers, but owing to the phenomena of what is known as electric osmosis, the current further acts to physically carry into the pores of the fibers, or to bodily impregnate said pores to any desired extent, with the said excess of aluminum hydrate and the latter is therefore deposited in said pores to a greater depth than it is possible to deposit it, through chemical precipitation alone. Nevertheless, I do not wish to limit myself to the simultaneous application of the metal acetate and the electric current.

It therefore follows that my product is easily distinguishable on the market from other products of a similar nature, in that it is much more resistant to the dissolving and frictional action of boiling water; and further, it even resists the solvent action of gasolene, benzene, and other similar hydrocarbon solvents, which no other like product will withstand so far as I have been able to discover.

In other words, it is evident that the electrolytic action of the current on the sodium palmitate and aluminum acetate solution will facilitate the chemical precipitation of both the aluminum palmitate and the aluminum hydrate, so that the rapidly traveling fabric will receive in a given time a greater quantity of each than would otherwise be the case. And as it is further evident that the quantity of water repelling hydrate or other compound which is formed from the soluble electrodes is independent of the strength of the said solution, it necessarily follows that my method may deliver a greater quantity of insoluble substances to the rapidly traveling fibers than it would be possible to deposit chemically thereon. And again, since the current acts to carry said excess, or additional quantity of substances bodily into the pores of the fibers, fabrics treated by my process still act to repel solvents seeking to enter said pores, even though the individual fibers may have been previously subjected to rather rough usage, which is not true of other similar products, so far as I have been able to find out. While, to the best of my knowledge and belief, the above correctly describes the chemical and electrical actions which take place in practice, yet, since said actions are by no means simple, or easily proved, it is to be understood that I do not limit myself

to any particular theory of operation or action.

While I have described one specific method of carrying out my invention, I do not desire, as I have pointed out, to be confined to any particular substances, values, or mechanisms used therein, since, as I have stated, they may be greatly varied without departing from the spirit of my invention.

10 Machines particularly adapted for use in practising my improved method are described in my pending application, Serial No. 9637, filed February 20, 1915, and in my application Serial No. 127,998 filed of even date herewith.

15 What I claim is:

1. The described method or process of waterproofing fibrous materials consisting in permeating the mass thereof with a saponaceous liquid and a metal acetate and electrolytically incorporating therein a metal palmitate and a metal hydroxid which coact in the fibers of the material being treated to make them of a non-capillary nature.

2. The described method of waterproofing fibrous materials, consisting in impregnating the mass with a saponaceous liquid and an aluminum acetate, and subjecting the material to the action of an electric current between the electrodes, one of which is soluble.

3. The described method of waterproofing fibrous materials, consisting in first impregnating the mass with a saponaceous liquid, then wetting with aluminum acetate simultaneous with the subjecting of the material to the action of an electric current between electrodes, one of which is soluble.

4. The described method of waterproofing fibrous materials, consisting in first impregnating the mass with a saponaceous liquid, 40 then wetting with an aluminum acetate, and simultaneously electrolytically depositing aluminum hydroxid in the fibers between electrodes, one of which is formed of aluminum.

5. The described method or process of waterproofing fibrous materials, consisting in first permeating or impregnating the mass thereof with a saponaceous substance, and then incorporating therein a metal acetate, 50 simultaneously with the subjecting of said impregnated fabric to the action of an electric current between aluminum electrodes to form a metal hydroxid.

6. The method of waterproofing fibrous materials, which consists in first impregnating said materials with an alkali metal palmitate, then simultaneously wetting with a metal acetate to form a metal hydroxid, and subjecting the impregnated fabric to 60 the action of a soluble anode in an electrolytic circuit, substantially as described.

7. The method of waterproofing fibrous materials, which consists in impregnating said materials with a solution of sodium palmitate and aluminum acetate to precipitate aluminum hydrate and palmitate; and subjecting said impregnated fabric to the action of an electric current between aluminum electrodes to produce an excess of 65 aluminum hydroxid and to drive the same into the fibers of said fabric, substantially as described.

ALFRED O. TATE.